

# UNITED STATES PATENT OFFICE.

IGNAZ KREIDL, OF VIENNA, AUSTRIA-HUNGARY.

## ENAMELING COMPOSITION.

1,104,679.

Specification of Letters Patent. Patented July 21, 1914.

No Drawing.

Application filed April 25, 1914. Serial No. 834,387.

*To all whom it may concern:*

Be it known that I, Dr. IGNATZ KREIDL, a subject of the Emperor of Austria-Hungary, resident of Vienna, in the Empire of Austria-Hungary, (whose post-office address is Kohlgasse 5-9, Vienna XXI,) have invented certain new and useful Improvements in Enameling Compositions, of which the following is a specification.

10 The invention relates to the manufacture of enameling compositions.

The invention is based upon the discovery that the metal compounds suitable as opaques such as the oxids and the silicates 15 of zirconium, tin, titanium and the like possess in colloidal state a great covering power, owing to the fact that colloids possess physical qualities which these compounds, in a non-colloidal (crystallloid) condition, do not 20 possess, which qualities aid in producing a satisfactory clouding action.

The invention consists therefore in the manufacture of enameling compositions in which as opaques are employed the 25 colloids of the metal compounds suitable as opaques, such as the oxids, the silicates of zirconium, tin, titanium and the like.

One method to render the oxids and silicates for example of zirconium suitable as opaques consists in finely grinding them and attacking them by means of acidulated or alkaline water (water containing acids, especially weak acids or alkaline matter). By such treatment the oxids and silicates become colloids. A colloidal formation as "sol" should be avoided by the presence of small quantities of crystalloids. The attack by the acid- or alkaline solutions 30 may be favored by the presence of clay.

In carrying the method into effect, the opaques such as an oxid or a silica-containing compound is ground in a mill in the presence of alkaline or acidulated water 45 with or without addition of small quantities of salts such as metallic salts, which by acting as electrolytes prevent the colloid forma-

tion as "sol"; the grinding process is continued until the opaques have become colloidal by the influence of the acidulated or alkaline water. In the manufacture of enameling composition the oxids or silicates employed as opaques may be ground in the mill simultaneously with the enamel mass in the presence of alkaline or acidulated 50 water. This method is less preferable, because the enamel mass should not be ground too fine and not too long as it may happen if grinding the enamel mass together with the opaques. 55

Other methods, of course, may be used for manufacture of the opaques, the essential feature consisting in that the opaques are obtained in a colloidal form. 60

The enameling composition is prepared in known manner. The enamel mass is melted and ground. The clouding agent is added to the already melted and ground mass. 65

What I claim is:

1. An enameling composition containing as an opaques a colloid of a metal compound suitable for opaques.

2. An enameling composition containing as opaques a colloid of an oxygen-containing metal compound suitable as opaques. 75

3. An enameling composition containing as opaques a colloid of a metal oxid suitable for opaques.

4. An enameling composition containing as an opaques a colloid of an oxygen-containing zirconium compound. 80

5. An enameling composition containing as opaques a colloid of an oxygen-containing zirconium compound. 85

In witness whereof I have hereunto signed my name in the presence of two subscribing witnesses.

DR. IGNATZ KREIDL.

Witnesses:

HUGO KEIK,  
AUGUST FUGGER.